

Patented Jan. 3, 1928.

1,654,628

# UNITED STATES PATENT OFFICE.

WELLS C. ADAMS, OF DETROIT, MICHIGAN.

## COMPOSITION OF MATTER.

No Drawing.

Application filed May 13, 1925. Serial No. 30,080.

This invention relates to a composition of matter to be used in the process of tone construction for modulating any tone produced by the horns, amplifiers or sound boards of 5 various kinds of instruments, for instance phonographs, radio sets and musical instruments. In the construction of these instruments materials are used for increasing and regulating tones, and my composition may 10 be applied to the materials, before or after being made into instruments, so that a desired quality or planing of tones may be attained.

It is a well known fact that many sound 15 emitting structures have surfaces which cause a commingling or confusion of sounds, and very often completely change the tone quality of a sound, for instance, by imparting a metallic or rasping tone to a sound that 20 would otherwise be melodious or natural. It is to such surfaces that my composition may be applied to eliminate any intermingling or confusion of sound, the composition affording a channel of transmission for 25 sounds so that each sound will be independent of the other, thus causing natural tones to be emitted without the same being effected by materials entering into the construction of the instrument.

30 My invention aims to provide a composition that may be applied similar to a varnish or paint, the composition forming a resilient or cushion surface that will prevent sound waves from being abruptly deflected or effected by the vibration of materials 35 forming the instrument from which the sounds are emitted. The composition may be applied to all surfaces of an instrument which in any manner whatsoever control the 40 quality of a tone emitted by the instrument, and the composition will be hereinafter more fully described and then claimed.

The composition consists of a mixture of 45 pure rubber, gutta percha, beeswax, linseed oil, varnish and litharge.

The rubber serves as a base or vehicle of the compound and is preferably pure and liquid emulsion in form. The gutta percha is ground to granular form, and in prepar-

ing the composition, I prefer to use the ingredients in about the following proportions:

|                      | Parts. |
|----------------------|--------|
| Rubber emulsion      | 20     |
| Gutta percha         | 2      |
| Beeswax              | 2      |
| Boiled linseed oil   | 1      |
| Non-volatile varnish | 4      |
| Litharge             | 3      |

In the above composition the rubber 60 emulsion contributes to a non-absorptive cushioning surface and the gutta percha contributes to the body of the composition in the formation of a coating.

The beeswax also contributes to the yieldingness of the surface formed by the composition and prevents the formation of a hard indurate sound rebounding surface. The linseed oil contributes to the drying of 70 the composition to a certain extent; the litharge prevents shrinking of the composition, and the varnish is used to finish off the surface and as a preservative.

Good results may be obtained by slightly 75 varying the parts of the composition, but I have found that a composition compounded in the proportions mentioned above produces a fine result after all the ingredients are mixed together, subjected to a heat of 80 approximately one hundred and fifty degrees F. for approximately twenty-four hours, and then placed in sealed containers for use at any time on the interior surface of any instrument channel or member which 85 emits sounds. A well known type of such sound emitting channel is a loud speaker forming part of the radio set. A great many of these loud speakers are made of wood and metal and it is such materials that 90 may be advantageously coated with my composition to impart the tone quality of the loud speaker. The composition will impart a surface to the loud speaker which will be flexible or resilient for sound deflecting purposes. This has been proven by extensive 95 use of the composition and while it has been primarily made for application to horns or loud speakers already in use, yet it may be

applied to materials entering into the construction of horns or sound boards.

What I claim is:—

1. A sound cushioning coating composition for sound reproducing instruments consisting of twenty parts fluid rubber, two parts beeswax, and an oil drier.
2. A sound cushioning coating composition for sound reproducing instruments consisting of fluid rubber, beeswax, and an oil drier.
- 10

3. A sound cushioning coating composition for sound reproducing instruments consisting of fluid rubber, beeswax, an oil drier, and varnish.

15  
4. A sound cushioning coating composition for sound reproducing instruments consisting of twenty parts fluid rubber, two parts beeswax, an oil drier, and varnish.

In testimony whereof I affix my signature.

WELLS C. ADAMS.